

Jan. 25, 1944.

G. J. H. DYKEMAN ET AL

2,340,048

METHOD OF TREATING YARNS WITH WAX

Filed May 12, 1942



FIG. 1.



FIG. 2.

Inventors

G. J. H. Dykeman

A. C. Goodings

J. C. Maybee

ATTY.

## UNITED STATES PATENT OFFICE

2,340,048

## METHOD OF TREATING YARNS WITH WAX

George J. H. Dykeman and Alfred C. Goodings,  
 Toronto, Ontario, Canada, assignors to Ontario  
 Research Foundation, Toronto, Ontario, Canada

Application May 12, 1942, Serial No. 442,710

13 Claims. (Cl. 8—155)

This invention relates to a method of treating yarns with wax to set the twist. More particularly, the invention relates to the specific method of application of the wax, that is the procedure followed in order to apply the wax to the yarn.

The object of the invention is to devise a simple practical method of treatment whereby the wax will be distributed uniformly over the whole length of the yarn without damaging or discolouring the yarn in the process.

In the process for setting twist using a wax emulsion described in co-pending application 426,070, A. C. Goodings and L. H. Turl, the treatment is restricted to the use of certain specified wax compositions and the process limited to rayon yarns. In the present case where molten wax is suitably employed, it has been found that the process can be usefully applied to other yarns in addition to rayon, for example nylon yarns. Further, the composition of wax which can be usefully employed is not so limited as in the emulsion treatment mainly by virtue of the fact that stability of emulsion is not a concern. Although compositions of wax consisting of paraffin wax with the addition of 10 to 20% of a solid mono- or di-glyceride such as stearic mono- or di-glyceride, have been found to be very suitable for use by the molten wax method of treatment, other compositions of wax might also be employed to give reasonably satisfactory results. There are of course certain properties in the wax composition which must be conformed to if the best results are to be obtained. For example the wax composition should have a melting point between 110° F. and 140° F. as outside limits and preferably should be between 115° F. and 130° F. It must not decompose at temperatures up to 160°; neither should it oxidise or show other undesirable changes on heating at this temperature for periods of 24 hours or longer. Certain physical characteristics of pliability and adhesiveness are desirable: a highly brittle type of wax for example would be unsatisfactory.

According to the present invention the yarn is treated with wax after being wound on a core or spool such as a spinning bobbin or in the form of a cone, and this application of wax is accomplished so that the distribution of the wax is uniform throughout the whole of the yarn. It is common practice to apply oil to yarn in a uniform manner by passing the strand of yarn over an oiled wick or oiling roller but such operation is slow and would be prohibitively cumbersome and difficult as well as time consuming and costly.

were it attempted with a wax. We have found however that yarn wound on a bobbin or cone can be treated with wax which will distribute itself uniformly throughout the convolutions of yarn on the bobbin. The conditions to be observed are important if satisfactory results are to be obtained.

The invention is hereinafter more particularly described, and apparatus for carrying out the same is illustrated diagrammatically in the accompanying drawing in which

Figure 1 is a perspective view of a tray for receiving the bobbins to be treated; and

Figure 2 a cross section of one of the troughs of the tray.

In the drawing like numerals of reference indicate corresponding parts in the different figures.

The method of treating the yarn after it has been twisted and wound on the spinning bobbins is as follows:

The bobbins containing the yarn are first given a pre-heating treatment at a temperature of 145° to 150° F. in a dry atmosphere for a period of 20 hours. This pre-heating treatment reduces the moisture content of the yarn and permits a more uniform distribution of the wax when this is later applied. After the preheating the bobbins are placed in separate troughs formed in a tray 2. Each trough contains a wick 4 having the required amount of wax 5 applied thereto for impregnating the yarn on one bobbin. Preferably the tray has twenty-four troughs 4. In the drawing a bobbin 3 is shown in only one of the troughs, for the sake of clarity and simplicity of illustration. Likewise, in the front corner trough only, a wick 4 is shown extending longitudinally of the bottom of the trough, and in an adjacent trough is shown the wick with the wax 5 added thereto.

When the bobbin of yarn is placed in the trough the wick and the outer convolutions of the yarn are in contact with one another longitudinally along a portion of the underside of the periphery of the wound yarn. It will be understood that the wick is merely a medium for bringing the wax into contact with the yarn and that direct contact between the wax and the outer convolutions of the yarn would be possible. For best results there should be contact between the periphery of the wound yarn and the wax substantially from one end to the other of the bobbin of yarn.

The trays containing the wax and yarn are then placed in the dry atmosphere of an oven

at a temperature of around 145° F. and left for a period of twenty-two hours. During this time the wax is absorbed through the wick and distributes itself uniformly over the whole of the yarn.

Following this treatment, the yarn is removed and conditioned for two hours in the moist atmosphere of a chamber having a dry bulb temperature of 155° F. and a wet bulb temperature of 152° F. After this conditioning the yarn on the spinning bobbins is ready for re-drawing and cone winding in the normal manner.

A similar procedure may be applied to yarn on bobbins before the twist has been inserted but in this case the final two hour conditioning in a warm moist atmosphere would not be carried out until after the twisting operation which in this case follows the application of the wax. Yarn on cones can also be treated according to this process although in general it is more desirable to treat the yarn before it is wound into cone form.

Emphasis has been laid on the necessity for obtaining a uniform distribution of wax over the yarn. Irregular distribution with consequent variation in behaviour of the yarn from place to place gives rise to serious trouble particularly in the case of high twist yarns to be used in the manufacture of hosiery. In order to obtain good, even, distribution of the wax it has been found preferable to give first an extended period of pre-heating to reduce the moisture content of the yarn to a low value. In the description given above, a preheating period of twenty hours at 145° to 150° F. is stated. This length of time might be somewhat reduced although to obtain good results with a fair degree of assurance, the twenty hour period is regarded as desirable.

To obtain uniform distribution of the wax throughout the whole of the yarn on the bobbin or cone, it has further been found necessary to permit the heating operation where the yarn and wax come together to extend over relatively long periods of time, for example twenty-two hours. At the temperature of 145° F. and using a normal sized spool containing 100 grams of yarn and to which 13% of its weight of wax is to be applied, about two hours is required for all the wax to be absorbed through the wick from the trough. The remainder of the heating period permits the wax to permeate the yarn throughout the bobbin and distribute itself in a uniform manner.

Higher temperatures than 145° F. may be employed but this is undesirable because of the effect of prolonging heating at these higher temperatures on both the wax and the yarn. Even though the absorption of the wax on to the yarn from the trough is found to be more rapid at the higher temperatures, the long time of heating is still required in order that the wax may distribute itself uniformly. For example, it was found that employing a temperature of 180° F. and heating for a period of five hours, portions of the yarn in the form of bands throughout the spool were to be observed in to which the wax had not penetrated. The observations on time and temperature indicate that a twenty hour heating period is probably a minimum for safety in obtaining good distribution of the wax.

The use of twenty-two hours as given in the procedure outlined above is a convenient length of time in that material on which the pre-heating operation is started one morning is ready for removal from the wax treating operation on the following morning. In certain cases longer peri-

ods, up to 36 hours in the heating chamber, may be found desirable. Wax which has been heated for long periods at a high temperature, for example 180° F., is adversely affected and can be observed to have developed a dark brown colour and is rendered more difficult in its removal in subsequent scouring operations.

The amount of wax to be applied to the yarn to give the best results is approximately 13% of the weight of the yarn. The application of too high a percentage of wax gives rise to trouble from the stripping of wax in subsequent operations: percentages over 15% give rise to this trouble. On the other hand, there is a lower limit to the amount of wax which can be used both from a point of view of adequate setting of the twist and also in obtaining uniform distribution. It has been found that percentages below 8% are more difficult to distribute uniformly throughout the yarn in the twenty-two hour heating period. It is possible that percentages below 8% may distribute themselves uniformly if the time of heating were still further prolonged although this is doubtful but longer lengths of time are not desirable from a point of view of mill operation.

Because of contact between the wax and the bobbin on which the yarn is wound, the use of metal bobbins is desirable. Suitable bobbins are those made of aluminium or stainless steel.

In the specification the expression "uniform distribution of the wax over the yarn" does not imply a mere surface coating. The wax impregnates the yarn, but the essential feature is not necessarily a uniform impregnation through each strand of yarn, but rather a uniform distribution of wax on the yarn throughout its length from the outer to the inner convolutions.

What we claim as our invention is:

1. Method of treating yarns with wax when wound on a core, which comprises subjecting the wax and the yarn while the wax and the outer convolutions of the yarn are in contact with one another longitudinally along a portion only of the periphery of the wound yarn to a temperature above the melting point of the wax for a period sufficient to permit the wax to distribute itself in a uniform manner throughout the whole length of yarn from the outer to the inner convolutions thereof.

2. Method of treating yarns with wax when wound on a core, which comprises preheating the yarn and then subjecting the wax and the yarn while the wax and the outer convolutions of the yarn are in contact with one another longitudinally along a portion only of the periphery of the wound yarn to a temperature above the melting point of the wax for a period sufficient to permit the wax to distribute itself in a uniform manner throughout the whole length of yarn from the outer to the inner convolutions thereof.

3. Method of treating yarns when wound on a core with wax having a melting point below 140° F., which comprises subjecting the wax and the yarn while the wax and the outer convolutions of the yarn are in contact with one another longitudinally along a portion only of the periphery of the wound yarn to a temperature of approximately 145° F. for a period sufficient to permit the wax to distribute itself in a uniform manner throughout the whole length of yarn from the outer to the inner convolutions thereof.

4. Method of treating yarns with wax when wound on a core, which comprises subjecting the wax and the yarn while the wax and the outer

convolutions of the yarn are in contact with one another longitudinally along a portion only of the periphery of the wound yarn to a temperature above the melting point of the wax for approximately twenty-two hours.

5. Method of treating yarns with wax when wound on a core, which comprises pre-heating the yarn at a temperature of about 145° F. to 150° F. for a period of approximately twenty hours and then subjecting the wax and the yarn while the wax and the outer convolutions of the yarn are in contact with one another longitudinally along a portion only of the periphery of the wound yarn to a temperature above the melting point of the wax for a period sufficient to permit the wax to distribute itself in a uniform manner throughout the whole length of yarn from the outer to the inner convolutions thereof.

6. Method of treating yarns when wound on a core with wax having a melting point below 140° F., which comprises pre-heating the yarn at a temperature of about 145° F. to 150° F. for a period of approximately twenty hours and then subjecting the wax and the yarn while the wax and the outer convolutions of the yarn are in contact with one another longitudinally along a portion only of the periphery of the wound yarn to a temperature of approximately 145° F. for a period sufficient to permit the wax to distribute itself in a uniform manner throughout the whole length of yarn from the outer to the inner convolutions thereof.

7. Method of treating yarns with wax when wound on a core, which comprises subjecting the wound yarn in contact along a portion only of its periphery with about 13% of its weight of wax to a temperature above the melting point of the wax for a period sufficient to permit the wax to distribute itself in a uniform manner throughout the whole length of yarn from the outer to the inner convolutions thereof.

8. Method of treating yarns with wax when wound on a core which comprises subjecting the yarn and wax having a melting point between about 110° F. and 140° F. while in contact with one another along a portion only of the periphery of the wound yarn to a temperature of approximately 145° F. for a period sufficient to permit the wax to distribute itself in a uniform manner throughout the whole length of yarn from the outer to the inner convolutions thereof.

9. Method of treating yarns with wax when

wound on a core which comprises subjecting the yarn and about 13% of its weight of wax having a melting point between about 110° F. and 140° F. while in contact with one another along a portion

5 only of the periphery of the wound yarn to a temperature of approximately 145° F. for a period sufficient to permit the wax to distribute itself in a uniform manner throughout the whole length of yarn from the outer to the inner convolutions thereof.

10. Method of treating yarns with wax when wound on a core, which comprises subjecting the wax and the yarn while in contact with one another along a portion only of the periphery of the wound yarn to a temperature above the melting point of the wax for a period sufficient to permit the wax to distribute itself in a uniform manner throughout the whole length of yarn from the outer to the inner convolutions thereof, and subsequently conditioning the yarn in a warm moist atmosphere.

11. Method of treating yarns with wax when wound on a core, which comprises placing the outer convolutions of the yarn in contact with a wick immersed in wax; and subjecting the yarn and the wax to a temperature above the melting point of the wax for a period sufficient to permit the wax to permeate the yarn and distribute itself in a uniform manner.

12. Method of treating yarn wound on a core, which comprises placing the core in a trough containing a wick immersed in a predetermined quantity of wax in such a manner that the under side of the outer convolutions of the yarn is in contact with the wick; and subjecting the yarn and wax to a temperature above the melting point of the wax for a period sufficient to permit the wax to permeate the yarn and distribute itself in a uniform manner.

13. Method of treating yarn wound on a core, which comprises placing the core in a trough containing a wick immersed in a predetermined quantity of wax in such a manner that the under side of the outer convolutions of the yarn is in contact with the wick; inserting the yarn in the trough in an oven; and subjecting the yarn and the wax to a temperature above the melting point of the wax for a period sufficient to permit the wax to permeate the yarn and distribute itself in a uniform manner.

GEORGE J. H. DYKEMAN.  
ALFRED C. GOODINGS.